

# UNITED STATES PATENT OFFICE

JAMES SPOONER HOWARD, OF MANSFIELD, ASSIGNOR TO HIMSELF, E. ADAMS, JR., OF ATTLEBOROUGH, T. E. GROVER, OF MANSFIELD, AND N. CARPENTER, OF ATTLEBOROUGH, MASSACHUSETTS.

## IMPROVEMENT IN ELECTROPLATING WITH ANTIMONY.

Specification forming part of Letters Patent No. 100,038, dated February 22, 1870.

*To all whom it may concern:*

Be it known that I, JAMES SPOONER HOWARD, of Mansfield, in the county of Bristol and State of Massachusetts, have invented a solution by which I can deposit antimony upon metals by electroplating; and I do hereby declare the following to be a full, clear, and exact description of my invention.

My solution is as follows: six (6) fluid ounces sulphate of ammonia; one-fourth ( $\frac{1}{4}$ ) fluid ounce cyanide potassa; eight (8) fluid ounces sulphate of antimony; one (1) gallon of water, (soft preferred.) Filter the whole.

These proportions may be varied from the exact quantities given; but they must be substantially as stated. When the solution is prepared the process of electroplating is the same as generally employed.

The advantage of electroplating with anti-

mony is, that I obtain a cheaper plate than by any other deposit.

I do not claim it as better, but simply as being cheaper and well adapted to plating many articles when it is desirable to save expense; neither do I claim any particular process of electroplating, as any known process will accomplish the purpose sought; but

What I claim as my invention, and desire to secure by Letters Patent, is—

The solution, substantially as given above, for electroplating with antimony.

In testimony whereof I have signed my name to this specification in the presence of two subscribing witnesses.

JAMES SPOONER HOWARD.

Witnesses:

CARROLL D. WRIGHT,

CHARLES F. BROWN.